

# UNITED STATES PATENT OFFICE.

THOMAS HOLLIDAY, OF HUDDERSFIELD, COUNTY OF YORK, ENGLAND.

## NAPHTHOL-DYED FABRIC.

SPECIFICATION forming part of Letters Patent No. 355,935, dated January 11, 1887.

Application filed September 15, 1886. Serial No. 213,627. (No specimens.)

*To all whom it may concern:*

Be it known that I, THOMAS HOLLIDAY, of Huddersfield, in the county of York, United Kingdom of Great Britain, have invented certain new and useful Improvements in the Treatment of Cotton or other Fiber, of which the following is a full, clear, and exact description.

This invention consists in the combination of cotton or other fiber with oxide or soap of lead and alpha or beta naphthol or coloring-matter formed with them, which is the result of the process described in the application for Letters Patent for "improvements in the treatment of cotton or other vegetable fiber," filed October 23, 1885, Serial No. 180,747.

The object of this invention is to produce cotton or other fiber upon which azo coloring-matter may be formed, and it is carried into effect by treating the fiber with a solution of a salt of lead in caustic alkali, and when a soap is required passing the said fiber through a soap solution or an emulsion, and, finally, treating the fiber thus prepared with naphthol in solution or suspension. A good method of accomplishing this result is to steep the fiber in a solution composed of ten pounds of acetate of lead in two hundred gallons of water, to which enough caustic soda has been added to precipitate all the lead and to redissolve the precipitate. In about thirty minutes the fiber may be washed, when it will be found to have fixed a considerable quantity of oxide of lead. It is then passed through a soap solution—say five pounds castile-soap in one hundred gallons of water—and, after again washing in water, the fiber will be found impregnated with lead soap.

The proportions may be varied, and other salts of lead or other alkali may be used. 40 Though a soap is preferred, an emulsion may be substituted when desired.

In preparing the fiber for the reception of the coloring-matters, it may be passed through a neutral solution of a salt of lead and afterward through a solution of caustic soda or potash; or the soluble soap may be mixed with a caustic alkali. The fiber, after having the oxide of lead or lead soap deposited upon it, is impregnated with a solution of, say, five 50 pounds of alpha or beta naphthol in one hundred gallons of warm water, and will then be ready for the formation of any azo coloring-matter having naphthol as a constituent. Those insoluble or nearly insoluble in water 55 are preferred; or the color may be formed simultaneously with the absorption of the naphthol, or in any other known manner.

The naphthol may be added to the bath of soluble soap and be absorbed by the fiber at 60 the time of the formation of the lead soap.

The fiber may be treated in the raw state or manufactured, and after treatment can be identified by the usual methods of analysis.

Having thus described my invention, what I 65 claim as new, and desire to secure by Letters Patent, is—

As a new and improved article of manufacture, the combination of cotton or other fiber with oxide or soap of lead and alpha or beta 70 naphthol, or coloring-matter formed with them, substantially as described.

THOMAS HOLLIDAY.

Witnesses:

EDWARD COCKSHAW,  
JOHN WILLIAM SYKES.